

(No Model.)

C. FISHER.

ANVIL.

No. 298,567.

Patented May 13, 1884.

*Fig. 1.*



*Fig. 2.*



*Fig. 3.*



WITNESSES:

*W. H. Culver*  
*John W. Lyle*

INVENTOR

*Clark Fisher*  
By his Attorneys,  
*W. C. Strawbridge*  
*Donald Taylor*

# UNITED STATES PATENT OFFICE.

CLARK FISHER, OF TRENTON, NEW JERSEY.

## ANVIL.

SPECIFICATION forming part of Letters Patent No. 298,567, dated May 13, 1884.

Application filed December 20, 1883. (No model.)

*To all whom it may concern:*

Be it known that I, CLARK FISHER, of Trenton, New Jersey, have invented certain Improvements in the Manufacture and Construction of Anvils, of which the following is a specification.

My invention relates to anvils of which the body is of cast metal and the face and horn covered with steel welded thereto.

Heretofore all anvils of the above character have been made by placing in the bottom of the mold first the steel plate which forms the face, and then the steel piece which forms the working-surface of the horn, the latter being placed with its broad endlapping partially over and resting upon the interior surface of the horn end of the face-plate, substantially as represented in Figure 1. When the mold is filled, the welding is accomplished by the sweeping of the molten iron over the interior or upwardly-projecting surfaces of the steel face-plate and horn-piece, as described in Re-issue No. 227 of the original patent granted to Mark Fisher and William Martin on October 16, 1847. Under the above conditions it is clear that the shoulder or depth of the horn-surface below that of the face of the completed anvil will be equal to the thickness of the steel used for the face-plate, and that the overlapped portions of the face-plate and horn-piece will not be welded, because their overlapping surfaces simply rest upon each other in the manner represented in Fig. 1, and prevent the access of molten metal between them.

In Fig. 2 is represented an anvil made by the method of which Fig. 1 is designed as an illustration, and the fact that there is no welding is indicated by a slight opening between the pen-lines. The thin unwelded part of the face-plate of anvils of the above construction is liable to crack off upon exposure to the hammer of the blacksmith. For many uses it is also desirable that the shoulder between the face and horn should be deeper than the thickness of the steel of the face-plate. Difficulties, however, in otherwise obtaining a perfect weld throughout the entire under surface of the face require that the steel face-plate should be thin, and this necessarily makes a low shoulder. Unless, on

the other hand, the two plates are arranged to lap upon each other, and thus form a close joint at the overlap, the molten iron escapes and flows out of the mold instead of filling it 55 and forming the anvil.

Generally stated, my invention is carried into practice by exposing the entire interior surface of the face-plate to the action of the molten iron without having any portion of it 60 in contact with the horn-steel, which is accomplished by leaving a space between the overlapping portions of the two plates vertically sufficient to admit the cast metal to flow between them, whereby a more perfect weld 65 of the contiguous extremities of these two pieces is obtained, which, as above explained, could not heretofore be secured on account of the exclusion of the molten welding metal from between the contact-surfaces to the entire distance or extent of the overlap.

In the manufacture of an anvil embodying my present improvement the molten metal is prevented from running through the open space between the plates by a dam either of 75 metal or sand core, or by a kindred suitable device, which can easily be arranged at the proper point within the mold by any practical molder.

In Fig. 3 of the drawings is represented an 80 anvil constructed according to my invention.

All of the figures of the drawings are longitudinal vertical central sectional elevations, any further description of which is unnecessary, except to say that A designates the body 85 of the anvil, B the face-plate, and C the horn-piece.

The advantages of my improvement reside not only in the securing of a more perfect weld throughout the extent of the face-plate, but 90 in securing a greater depth of shoulder, as at S in Fig. 3, and in preventing the liability of fracture in the front portion of the face-plate.

It is proper to add that the face-plates may, if desired, be made of wrought-iron instead of 95 steel.

Having thus described my invention, I claim and desire to secure by Letters Patent—

An anvil having a steel face-plate and a steel or wrought-iron plate covering the horn, 100 the union being effected by casting the iron body on the plates, in which the adjacent ex-

tremities of the horn-piece and face-plate are one above the other, and out of contact with each other, and in which the cast metal extends under the entire surface of the face-plate, and between the end thereof nearest to the horn and the horn piece or plate, substantially as and for the purposes set forth.

In testimony whereof I have hereunto signed my name this 14th day of December, A. D. 1883.

CLARK FISHER.

In presence of—

JOHN JOLLEY, Jr.,  
F. NORMAN DIXON.